

## UNITED STATES PATENT OFFICE.

MICHAEL G. MINAEFF AND ALBERT PARSONS SACHS, OF NEW YORK, N. Y., ASSIGNEES,  
BY MESNE ASSIGNMENTS, TO THE LARVEX CORPORATION, OF BROOKLYN, NEW  
YORK, A CORPORATION OF NEW YORK.

## ART OF MOTHPROOFING.

No Drawing.

Application filed June 21, 1924. Serial No. 721,529.

This invention is a moth proofing composition and one of the objects of the invention is to provide an effective moth proofing treatment for finished fabrics, knitted goods and the like and one particularly suited to household use and to the treatment of finished fabrics after they leave the mill and before or after making such fabrics into clothing. We have found that most of the difficulties of prior practice have been due to the use of solutions containing too strong an acid such as sulphuric acid or too large quantities of weaker acids. When strong acids or large quantities of the weaker acids are used, it is essential that the material treated be subsequently thoroughly washed or rinsed; otherwise the material will remain strongly acid and will be subject to deterioration and loss of tensile strength due to the presence of this acid.

In the treatment of finished goods or clothing, it is not, manifestly, feasible or practical to rinse or wash the goods after treatment to remove surplus acid and accordingly the present invention aims to produce a composition with which finished goods and clothing may be treated to leave them in a substantially neutral or only very slightly acid condition and without necessitating any subsequent treatment such as washing, rinsing or the like.

Another object of the invention is to provide a moth proofing treatment which will be satisfactorily permanent against wear, usage, cleaning, wetting by rain, etc.

A still further object of the invention is to provide a composition which may be efficiently and properly applied to woolens by spraying or sponging them with the composition. It has been found that solutions of fluorides combined with other chemicals having moth proofing properties do not easily penetrate into woolen fabrics and when applied in pure form are apt to roll off or evaporate without impregnating the fabrics. Impregnation of a fabric by a moth proofing solution cannot always be readily accomplished even if the fabric can be immersed in the solution for a short time, but, as even this is not practical in the treatment of finished garments, the composition of this invention is so constituted that it will of itself effect efficient wetting of the fabric without immersion.

An important feature of the present invention resides in the fact that the moth proofing composition of the present invention is practically neutral or only very slightly acid in reaction and exhibits no deleterious properties toward the animal fibers. At the same time, it retains the desirable moth proofing properties and may be prepared in such form that it can be readily used alike by the textile trade and housewives with the same efficient and effective results in protecting woolen goods from the ravages of the moth larvæ.

Our research and experiments have demonstrated that a moth proofing composition containing soluble fluorides or soluble silico fluorides or mixtures of these soluble fluorides and silico fluorides can be prepared in such strength in aqueous solution as to impart to the resulting composition properties well adapted to carry out the objects of the invention which have been enumerated.

It has been found that certain organic compounds applied alone or in a mixture with one another, or with fluorides or with silico fluorides, or both, show valuable moth proofing properties. Among these organic compounds are the alkali metal salts of benzene sulphonic acids, or of derivatives of benzene sulphonic acid; for example: sodium benzene sulphonate, sodium chlor-benzene sulphonate or sodium benzene di-sulphonate—the function of any one of these salts being to enhance the moth proofing effect of the composition.

Another organic compound which may be employed is a salt of naphthalene beta-sulphonic acid or of its derivatives, as for example: sodium, potassium, lithium or barium salt of chlor-naphthalene-beta-sulphonic acid, or of chlor-naphthalene-beta-di-sulphonic acid; the function of such salt being to materially enhance the moth proofing effect of the composition to which it is added.

In our compositions we may use a soluble sulphate, i. e., sodium sulphate or alum, which we have found assists materially in the wetting of the fabrics and increases the permanency of the moth proofing effect.

A moth proofing composition comprising the ingredients enumerated produces very satisfactory results when applied to woolen goods for the purpose of moth proofing the same in that the goods so treated are found

to be immune to the attacks of the moth larvae and do not show any deterioration or weakening of tensile strength or durability of the fibers or fabrics subsequent to this treatment with such a composition.

It has been found in practice that the ingredients entering into our composition can be used within the following definite ranges: sodium fluoride, .1 to 2.5%; sodium silico fluoride, .1 to .6%; sodium sulphate, .1 to 1%; sodium benzene sulphonate, .01 to .5%; sodium salt of naphthalene beta-sulphonic acid, .01 to .4%; and alum, up to .5%.

15 It is of course to be understood that neither all the maximum quantites nor all the minimum quantites given in this formula should be compounded, but we have set forth the practical limits of the respective constituents which enter into the composition.

We usually prefer to employ the ingredients enumerated with the omission of alum when sodium fluoride is used, whereas if 25 the sodium fluoride is omitted, the alum is generally employed.

It is important from a practical standpoint that woolens treated with our composition do not require washing or rinsing as 30 in the case of prior processes where fluorides are applied in strongly acidic solutions.

By the term "soluble fluoride" we mean to include the fluorides of the alkali metals, sodium, potassium, and lithium, and the 35 metals zinc and aluminum.

By the term "soluble silico fluoride" we mean to include the silico fluorides of the alkali metals, sodium, potassium, lithium, and the metals zinc and aluminum.

40 The term "alkali metal salt of benzene sulphonic acid" is intended to include also such salts of derivatives of such acid.

The term "a metal salt of naphthalene beta-sulphonic acid" is intended to include 45 the sodium, potassium, lithium, and barium salt of the substituted and unsubstituted acid.

The term "a soluble sulphate" is intended to include the alkali metal sulphates as well 50 as zinc and aluminum sulphates, and potash alum.

It is of commercial practical importance that the moth proofing composition which we have hereinbefore described will not appreciably act on glass and this renders it possible to package the composition for household use in bottles in which it may be kept indefinitely and ready for use.

Having thus fully described the invention, 60 what we claim as new and desire to secure by Letters Patent is:

1. A substantially neutral moth proofing composition containing a soluble silico fluoride.

65 2. A substantially neutral moth proofing

composition containing sodium silico fluoride.

3. A substantially neutral moth proofing composition containing a soluble silico fluoride and a soluble sulphate. 70

4. A moth proofing composition containing a soluble fluoride, a soluble silico fluoride, and a soluble sulphate.

5. A moth proofing composition containing a soluble fluoride, a soluble silico fluoride, a soluble sulfate, and an alkali metal salt of benzene sulphonic acid. 75

6. A moth proofing composition containing a soluble fluoride, a soluble silico fluoride, a soluble sulfate, an alkali metal salt of benzene sulphonic acid, and a metal salt of naphthalene beta-sulphonic acid. 80

7. A moth proofing composition containing sodium fluoride, sodium silico fluoride, and sodium sulfate. 85

8. A moth proofing composition containing sodium fluoride, sodium silico fluoride, sodium sulfate, and sodium benzene sulfonate.

9. A moth proofing composition containing sodium fluoride, sodium silico fluoride, sodium sulfate, sodium benzene sulfonate, and sodium naphthalene beta-sulphonate. 90

10. A moth proofing composition containing sodium fluoride approximately .1 to 2.5%, sodium silico fluoride approximately .1 to .6%, and sodium sulfate approximately .1 to 1%. 95

11. A moth proofing composition containing sodium fluoride approximately .1 to 2.5%, sodium silico fluoride approximately .1 to .6%, sodium sulfate approximately .1 to 1%, and sodium benzene sulfonate approximately .01 to .5%. 100

12. A moth proofing composition containing sodium fluoride approximately .1 to 2.5%, sodium silico fluoride approximately .1 to .6%, sodium benzene sulfonate approximately .01% to .5%, and sodium naphthalene beta-sulfonate approximately .01 to 4%. 110

13. A moth proofing composition containing sodium fluoride approximately .1 to 2.5%, and sodium silico fluoride approximately .1 to .6%. 115

14. The method of moth proofing woolen goods which consists in applying a substantially neutral liquid composition containing sodium silico fluoride and a soluble sulphate. 120

15. The method of moth proofing woolen goods which comprises applying a substantially neutral composition containing a soluble fluoride and a soluble silico fluoride thereto. 125

16. The method of moth proofing woolen goods which comprises applying a substantially neutral composition containing a soluble fluoride, a soluble silico fluoride, and a soluble sulfate thereto. 130

17. The method of moth proofing woolen

goods which comprises applying a composition containing a soluble fluoride, a soluble silico fluoride, a soluble sulfate, and an alkali metal salt of benzene sulphonic acid, and a metal salt of naphthalene beta-sulphonic acid thereto.

18. The method of moth proofing woolen goods which comprises applying a composition containing a soluble fluoride, a sol-

uble silico fluoride, a soluble sulfate, an alkali metal salt of benzene sulphonic acid, <sup>10</sup> and a metal salt of naphthalene beta-sulphonic acid thereto.

In testimony whereof we have signed the foregoing specification.

MICHAEL G. MINAEFF.

ALBERT PARSONS SACHS.